

## UNITED STATES PATENT OFFICE.

MARIUS LATOUR, OF PARIS, FRANCE, ASSIGNOR TO LATOUR CORPORATION, OF JERSEY CITY, NEW JERSEY, A CORPORATION OF DELAWARE.

## ELECTRIC COIL CONSTRUCTION.

No Drawing. Application filed May 17, 1923, Serial No. 639,708, and in France June 14, 1922.

In my copending application Serial No. 493,677 filed August 19, 1921, it has been pointed out that an alloy made up of iron, nickel, and manganese may be particularly suited, when chosen in appropriate proportions, for the construction of magnetic circuits in static multiplier devices for high frequency currents. Now, the relative quantities that have been found to give good results, after exhaustive testing, are about as follows: 33.92% nickel and 1.15% manganese. The permeability of these alloys decreases notably with the temperature, so that one operates preferably at about a temperature of 100 degrees C. As a matter of fact, it has been found in the case of the alloys in question, that an increase in temperature tends to greatly diminish the losses due to hysteresis. Moreover, these latter losses increased by the use of sheets of great thinness are reduced to a low value if care is taken to anneal the laminations of the alloy in question in vacuo. The resistivity is of an order of magnitude around 85 microhms per cubic centimeter.

Multiplier devices built with these alloys can naturally be used also for the purpose of multiplying the frequency of a current of less value than hereinbefore considered, as obtained, e. g., by a Poulsen or a mercury-arc.

In the copending application the proposition has been made to use in loading coils or Pupin coils a similar alloy. This alloy, as a matter of fact, occasions but very small 35 losses; but since in reality the sheets thereof are annealed in vacuo, the permeability in the initial inductions is by far greater than in ordinary iron. One would thus be led to use the gaps that have been provided even 40 while using the same alloy.

Another application of this alloy would be to employ it in the construction of the magnetic circuit of high-frequency transformers used in combination with amplifiers. 45 In transformers of this sort it is, as a matter of fact, very desirable to reduce the losses to a minimum, particularly so in resonance amplifiers. It may thus be of advantage to substitute in these amplifier transformers 50 this alloy for iron itself the use of which has been proposed in French Patent No. 512,295 of the present inventor.

Having described my invention, what I claim is:

A composition of matter forming the magnetic circuit of an electrical device, comprising substantially 33.9 per cent nickel, 1.15 per cent manganese, and iron, whereby electrical losses are reduced to a minimum. 60

MARIUS LATOUR.